# EUROPEAN PATENT SPECIFICATION

(11) **EP 3 424 738 B1**
(45) Date of publication and mention of the grant of the patent: **13.09.2023**
(21) Application number: 17179248.4
(22) Date of filing: 03.07.2017
(51) Int. Cl.: B41M 1/04, B41M 1/30

(54) **PROCESS FOR PRINTING INK TO PROVIDE HIGH OPACITY SUBSTRATE**
VERFAHREN FÜR DRUCKFARBE ZUR BEREITSTELLUNG EINES SUBSTRATS MIT HOHER OPAZITÄT
PROCÉDÉ D'ENCRE D'IMPRESSION POUR OBTENIR UN SUBSTRAT DE HAUTE OPACITÉ

(43) Date of publication of application: 09.01.2019
(73) Proprietor: The Procter & Gamble Company, Cincinnati, OH 45202 (US)
(72) Inventor: KOHLWEYER, Christian, 65824 Schwalbach am Taunus (DE); BLUM, Thorsten, 65824 Schwalbach am Taunus (DE); BAKER, Paul Edmund, Egham, Surrey TW20 9NW (GB)
(74) Representative: P&G Patent Germany

(56) References cited:
- EP-A1- 1 857 290
- EP-A2- 1 249 345
- WO-A2-2007/029194

## Description

### Field of the Invention

The present invention relates to a process for printing of ink onto a polymeric film substrate. The process provides a high opacity printed substrate.

### Background of the Invention

Consumer products are typically packaged by the product manufacturer and shipped in packaged form through a distribution network to the consumers. In many cases consumers make their choice about which products to buy based, at least in part, on the information communicated by, and the overall impression given by, the package appearance.

Certain consumer products, such as absorbent hygiene articles, are packaged and presented to consumers in a printed plastic film which is folded and sealed so as to contain the products.

These products are thus protected from contamination as they pass through the distribution network into the hands of the consumers. Printed graphics and text on the package convey to the consumer information about the product.

Manufacturers are seeking to use thinner plastic films for packaging partly in response to demands for ever more lightweight packaging which has the advantage of improved environmetal sustainability profile. Another advantage of lightweight packaging is lower packaging material costs.

A disadvantage of thin plastic films for packaging is that reduced thickness leads to reduced opacity of the film. The point may be reached where the plastic film is so thin that the product within the package is at least partly visible from the outside. This undesirable effect may be exacerbated when the plastic film is white or a pale or pastel colour and when the packaged products within the package are themselves decorated with bright, vivid colours. In this case the colours of the product or the outline of the products may be visible through the thin packaging film.

EP-1 857 290, published on November 21^{st} 2007, discloses opaque printed substrates that can be made with clear or low opacity films. Metallic ink is used in the preparation of the opaque printed substrate.

There remains a need for opaque printed substrates which mask the outline and the colours of the products which are contained within a package which is made from the opaque printed substrate even when the printed substrate comprises a thin polymeric film, for example of thickness of 100 micrometers or less.

### Summary of the Invention

The present invention relates to a process for flexographic printing of ink onto a thin polymeric film substrate. In particular the process relates to printing using a central impression cylinder press, wherein the width of printed substrate is greater than 800 mm, to provide a high opacity printing process. According to the present invention the printing process comprises: transferring ink from an ink reservoir to an anilox roll; transferring the ink from the anilox roll to a printing plate; and applying the ink to the surface of the substrate by applying pressure between the printing plate and an impression surface and passing the substrate between the printing plate and the impression surface; wherein the ink is white ink comprising pigment selected from the group consisting of: titanium dioxide, zinc oxide, lithopone and zinc sulfide; wherein the thickness of the polymeric film substrate is from 12 to 100 micrometers and the ink volume transferred by the anilox roll is from 9-20 cm³/m², and wherein the printing plate is a high definition printing plate comprising at least 40 lines per centimeter, wherein the high definition printing plate comprises an array of dots which are round top dots with microcell structures; wherein the opacity of the polymeric film substrate before the printing process, measured according to ISO 6504-03, is less than 80% and the opacity of the printed film substrate after printing of the white ink is greater than 92%, measured according to ISO 6504-03.

### Brief Description of the Drawings

Figure 1 shows a schematic of a flexographic printing system.
Figure 2 shows in more detail a part of Figure 1.

### Detailed Description of the Invention

### Definitions

"Flexography" is a form of printing that uses flexible rubber relief plates. It is commonly used in package printing.

"Anilox" is an engraved metal or ceramic roller used in flexographic printing presses to transfer ink from the fountain roller (or directly from the fountain) to the printing plate. A flexographic inking system is sometimes known as an anilox system. The purpose of the anilox roller is to pick up ink from the fountain roller (or, in some configurations, directly from the ink fountain) and deliver a predetermined, metered, uniform amount of ink to the rubber printing plate.

"Plate Cylinder" is the part of the flexographic press to which the rubber or photopolymer plate is attached. The flexo plate cylinder can be removed and swapped with cylinders of varying diameters, depending upon the application. The plate is inked by the adjacent anilox roller, and transfers the raised images directly to the web of substrate passing between the plate cylinder and the impression cylinder.

A central impression press is a type of printing press used in multi-color flexography in which a single large-diameter common impression cylinder supports the substrate as it contacts a series of adjacent plate cylinders, which lay down successive colors to the left or right dependent on the web feed direction. Central impression presses can have at least two printing units, with six to ten being the most common.

The opaque printed substrate typically serves as a "blank canvas" onto which coloured inks are then printed in order to create the final package comprising printed graphics, text etc. The process according to the present invention provides an opaque printed substrate which is particularly suitable for receiving coloured inks subsequently printed thereon. Without wishing to be bound by theory, it is believed that the dry opaque printed substrate, preferably white printed substrate, has a relatively high surface roughness which provides a desirable matte effect. Moreover the high opacity printed substrate helps to reduce or avoid undesirable interaction between the coloured graphics on the outside of the package and the coloured products which are partly visible from within the package. This helps to maintain the bright and vibrant appearance of the package graphics and avoids a dull appearance that may otherwise be caused by the coloured products lying behind the coloured graphics.

From finger printing tests, it was observed that printing the coloured inks onto the opaque printed substrate results in an improved ink lay-down with no pinholes in solid areas, smooth print outs of vignettes with no ink bridging, cleaner print which helps deliver sharper printed dots in highlight areas and a wider colour gamut.

Inks are solvent-based inks which typically comprise, pigment, resin, solvent and additives.

White inks used in the present invention use titanium dioxide, zinc oxide, lithopone or zinc sulfide as white pigment. Titanium dioxide is preferred as white pigment. Titanium dioxide exists in three different crystalline forms, rutile, anatase and brookite. The rutile and anatase forms have the highest refractive index of all white pigments, and provide the highest coverage for ink coatings. Rutile has the greatest opacity, and anatase has the greatest whiteness. The anatase form is most preferred. Pigments are typically subject to modification by grinding and/or surface treatment, for example. Grinding may modify surface area, with higher surface areas generally preferred. Resins may comprise nitrocellulose, preferably in combination with polyurethane or polyacrylate.

Solvents may comprise ethanol or isopropyl alcohol, or combinations thereof. Preferred solvents are mixtures of ethanol or isopropyl alcohol, or combinations thereof, with an acetate such as ethyl acetate or n-propyl acetate. Other solvents include various glycol ethers.

Various additives may be added to the ink composition, such as wax.

Figure 1 shows a schematic of a flexographic printing system comprising ink supply (10), anilox roller (20), print cylinder (30) and impression cylinder (40).

The ink supply (10) may be a chambered doctor blade system, preferably comprising a hard doctor blade and set to a doctor blade chamber pressure of from 1 to 4 bar.

The anilox roller (20) serves to meter the volume of ink which is applied. Preferably, the outer surface (22) of the anilox roller comprises an array of cavities or "cells" (24) arranged from 100-250 lines per centimeter. The cells may be hexagonal in shape. Alternatively anilox rollers may also be used which do not comprise discrete cells such as High Volume Solids, Tri-Helical, Fluid, Open Channel and Open Slalom Ink Channel anilox engraved geometries.

Printing plate (32) is disposed around the plate cylinder (30). The printing plate is a high definition printing plate comprising an array of dots which are round top dots with microcell structures.

Impression surface (42) is disposed around the impression cylinder (40).

Polymeric film substrate (50) is passed between the printing plate (32) and the impression surface (42). Pressure is applied between the printing plate and the impression surface. Preferably the applied pressure is from 80-220 N/m². Preferably the speed at which the substrate is passed between the printing roll and the impression roll is from 100-600, preferably from 150-300 meters/minute.

The polymeric film substrate preferably comprises low density polyethylene, high density polyethylene, Polypropylene, bi-orientated Polypropylene, other combinations of polyolefins, polyethylene terephthalate (polyesters), metallised polyesters and nylon.

The polymeric film substrate may be either a pigmented film or a clear film.

The quality of the package impression may be further improved by printing with high resolution graphics. Preferably graphic images should be created and maintained in high resolution. For example photographic images may be captured and stored using at least 50 megaPixels. Preferably the high resolution images are maintained in master data files so as to minimize degradation of image quality over time through repeated digital manipulation.

### Examples:

| | White Ink Reference | White Ink High Opacity |
|---|---|---|
| Pigment | Titanium dioxide | Titanium dioxide |
| Resin | Nitrocellulose/ Polyurethane | Nitrocellulose/ Polyacrylate |
| Solvent | Ethanol/ Propylene Glycol Ether, ratio 3:1 | Ethanol/ Ethyl Acetate, ratio 4:1 |

A pigmented film substrate having a starting opacity of 80% was subjected to a flexographic printing process as set out above applying high opacity white ink comprising titanium dioxide, nitrocellulose, polyacrylate, ethanol and ethyl acetate. The opacity was increased to 92%.

Opacity was measured using an X-Rite advance spectrophotometer according to ISO 6504-03. The dimensions and values disclosed herein are not to be understood as being strictly limited to the exact numerical values recited. Instead, unless otherwise specified, each such dimension is intended to mean both the recited value and a functionally equivalent range surrounding that value. For example, a dimension disclosed as "40 mm" is intended to mean "about 40 mm".

## Claims

1. A process for flexographic printing of ink onto a polymeric film substrate in a central impression cylinder press, wherein the width of printed substrate is greater than 800 mm, to provide high opacity printing, the printing process comprising:
transferring ink from an ink reservoir to an anilox roll;
transferring the ink from the anilox roll to a printing plate; and
applying the ink to the surface of the substrate by applying pressure between the printing plate and an impression surface and passing the substrate between
the printing plate and the impression surface;
wherein the ink is white ink comprising pigment selected from the group consisting of: titanium dioxide, zinc oxide, lithopone and zinc sulfide;
wherein the thickness of the polymeric film substrate is from 12 to 100 micrometers and the ink volume transferred by the anilox roll is from 9-20 cm³/m², and
wherein the printing plate is a high definition printing plate comprising at least 40 lines per centimeter, wherein the high definition printing plate comprises an array of dots which are round top dots with microcell structures; wherein the opacity of the polymeric film substrate before the printing process, measured according to ISO 6504-03, is less than 80% and the opacity of the printed film substrate after printing of the white ink is greater than 92%, measured according to ISO 6504-03.

2. The process according to claim 1 wherein the anilox roll comprises lines of cells between 100 and 250 lines per centimeter.

3. The process according to either of the previous claims wherein the speed at which the substrate is passed between the printing roll and the impression roll is from 100-500 meters/minute, preferably from 150-300 meters/minute.

4. The process according to any of the previous claims wherein the print pressure applied between the printing roll and the impression roll is from 80-220 N/m².

5. The process according to any of the previous claims wherein the ink comprises pigment, resin and solvent, and wherein the pigment comprises titanium dioxide.

6. The process according to claim 5 wherein the solvent comprises ethanol or isopropyl alcohol, or mixtures thereof.

7. The process according to claim 6 wherein the solvent further comprises an acetate, preferably an acetate selected from ethyl acetate or n-propyl acetate or mixtures thereof.

8. The process according to either of claims 6 or 7 wherein the solvent further comprises glycol ether.

9. The process according to any of claims 5 to 8 wherein the resin comprises nitrocellulose.

10. The process according to claim 9 wherein the resin further comprises polyurethane or polyacrylate, or mixtures thereof.

## Patentansprüche

1. Verfahren zum Flexographiedrucken von Tinte auf ein Polymerfoliensubstrat in einer zentralen Gegendruckzylinderpresse, wobei die Breite des gedruckten Substrats größer als 800 mm ist, um einen Druck mit hohet Trübung bereitzustellen, das Druckverfahren umfassend:
Übertragen von Tinte von einem Tintenbehälter auf eine Anilox-Walze;
Übertragen der Tinte von der Anilox-Walze auf eine Druckplatte; und
Aufbringen der Tinte auf die Oberfläche des Substrats durch Aufbringen von Druck zwischen der Druckplatte und einer Bedruckungsoberfläche und Leiten des Substrats zwischen der Druckplatte und der Bedruckungsoberfläche;
wobei die Tinte weiße Tinte ist, umfassend ein Pigment, ausgewählt aus der Gruppe bestehend aus: Titandioxid, Zinkoxid, Lithopone und Zinksulfid;
wobei die Dicke des Polymerfoliensubstrats von 12 bis 100 Mikrometer beträgt und das Tintenvolumen, das von der Anilox-Walze übertragen wird von 9-20 cm³/m² beträgt, und
wobei die Druckplatte eine Hochauflösungsdruckplatte ist, umfassend mindestens 40 Zeilen pro Zentimeter, wobei die Hochauflösungsdruckplatte eine Anordnung von Punkten umfasst, die runde obere Punkte mit Mikrozellstrukturen sind;
wobei die Trübung des Polymerfoliensubstrats vor dem Druckverfahren, gemessen nach ISO 6504-03, weniger als 80 % und die Trübung des gedruckten Foliensubstrats nach dem Drucken der weißen Tinte größer als 92 % ist, gemessen gemäß ISO 6504-03.

2. Verfahren nach Anspruch 1, wobei die Anilox-Walze Zeilen von Zellen zwischen 100 und 250 Zeilen pro Zentimeter umfasst.

3. Verfahren nach einem der vorstehenden Ansprüche, wobei die Geschwindigkeit, mit der das Substrat zwischen der Druckwalze und der Bedruckungswalze geleitet wird, von 100 bis 500 Meter/Minute, vorzugsweise von 150-300 Meter/Minute, beträgt.

4. Verfahren nach einem der vorstehenden Ansprüche, wobei der Druck beim Drucken, der zwischen der Druckwalze und der Bedruckungswalze aufgebracht wird, von 80-220 N/m² beträgt.

5. Verfahren nach einem der vorstehenden Ansprüche, wobei die Tinte ein Pigment, ein Harz und ein Lösungsmittel umfasst und wobei das Pigment Titandioxid umfasst.

6. Verfahren nach Anspruch 5, wobei das Lösungsmittel Ethanol oder Isopropylalkohol oder Mischungen davon umfasst.

7. Verfahren nach Anspruch 6, wobei das Lösungsmittel ferner ein Acetat, vorzugsweise ein Acetat, ausgewählt aus Essigsäurethylester oder n-Propylacetat oder Mischungen davon, umfasst.

8. Verfahren nach einem der Ansprüche 6 oder 7, wobei das Lösungsmittel ferner Glykolether umfasst.

9. Verfahren nach einem der Ansprüche 5 bis 8, wobei das Harz Cellulosenitrat umfasst.

10. Verfahren nach Anspruch 9, wobei das Harz ferner Polyurethan oder Polyacrylat oder Mischungen davon umfasst.

## Revendications

1. Procédé d'impression flexographique d'encre sur un substrat de film polymère dans une presse à cylindre d'empreinte centrale, dans lequel la largeur de substrat imprimé est supérieure à 800 mm, pour fournir une impression d'opacité élevée, le procédé d'impression comprenant :
le transfert d'encre d'un réservoir d'encre à un rouleau tramé ;
le transfert de l'encre du rouleau tramé à une plaque d'impression ; et
l'application de l'encre à la surface du substrat en appliquant une pression entre la plaque d'impression et une surface d'empreinte et en passant le substrat entre la plaque d'impression et la surface d'empreinte ;
dans lequel l'encre est une encre blanche comprenant un pigment choisi dans le groupe constitué par : le dioxyde de titane, l'oxyde de zinc, la lithopone et le sulfure de zinc ;
dans lequel l'épaisseur du substrat de film polymère est de 12 à 100 micromètres et le volume d'encre transféré par le rouleau tramé est de 9 à 20 cm³/m², et
dans lequel la plaque d'impression est une plaque d'impression haute définition comprenant au moins 40 lignes par centimètre, dans lequel la plaque d'impression haute définition comprend un réseau de points qui sont des points supérieurs ronds avec des structures de microcellules ;
dans lequel l'opacité du substrat de film polymère avant le procédé d'impression, mesurée selon ISO 6504-03, est inférieure à 80 % et l'opacité du substrat de film imprimé après impression de l'encre blanche est supérieure à 92 %, mesurée selon ISO 6504-03.

2. Procédé selon la revendication 1 dans lequel le rouleau tramé comprend des lignes de cellules entre 100 et 250 lignes par centimètre.

3. Procédé selon l'une ou l'autre des revendications précédentes dans lequel la vitesse à laquelle le substrat est passé entre le rouleau d'impression et le rouleau d'empreinte est de 100 à 500 mètres/minute, de préférence de 150 à 300 mètres/minute.

4. Procédé selon l'une quelconque des revendications précédentes dans lequel la pression d'impression appliquée entre le rouleau d'impression et le rouleau d'empreinte est de 80 à 220 N/m².

5. Procédé selon l'une quelconque des revendications précédentes dans lequel l'encre comprend un pigment, une résine et un solvant, et dans lequel le pigment comprend du dioxyde de titane.

6. Procédé selon la revendication 5 dans lequel le solvant comprend de l'éthanol ou de l'alcool isopropylique, ou des mélanges de ceux-ci.

7. Procédé selon la revendication 6 dans lequel le solvant comprend en outre un acétate, de préférence un acétate choisi parmi l'acétate d'éthyle ou l'acétate de n-propyle ou des mélanges de ceux-ci.

8. Procédé selon l'une quelconque des revendications 6 ou 7 dans lequel le solvant comprend en outre de l'éther de glycol.

9. Procédé selon l'une quelconque des revendications 5 à 8 dans lequel la résine comprend une nitrocellulose.

10. Procédé selon la revendication 9 dans lequel la résine comprend en outre un polyuréthane ou un polyacrylate, ou des mélanges de ceux-ci.
